

# UNITED STATES PATENT OFFICE.

LEONHARD LEDERER, OF SULZBACH, GERMANY.

## PRODUCT RESEMBLING CELLULOID AND PROCESS FOR PRODUCING THE SAME.

1,195,040.

Specification of Letters Patent. Patented Aug. 15, 1916.

No Drawing. Application filed May 2, 1907, Serial No. 371,533. Renewed July 1, 1916. Serial No. 107,150.

To all whom it may concern:

Be it known that I, Dr. LEONHARD LEDERER, a subject of the Emperor of Germany, residing at Sulzbach, Germany, have invented certain new and useful Chemical Products Resembling Celluloid and Process for Producing the Same, of which the following is a specification.

In the manufacture of celluloid camphor has hitherto been generally used as one of the principal ingredients, although many attempts have been made to find a cheaper substitute and to render celluloid less inflammable by the addition of other materials.

I have discovered that chloral-hydrate, chloral-alcoholate and similar materials as well as mixtures of the same are eminently suitable to replace camphor. The products thus obtained resemble celluloid in every essential respect and are moreover less inflammable. They may, of course, contain some of the admixtures usually found in celluloid, and instead of nitro-cellulose organic acid esters of nitro-cellulose or mixtures of nitro-cellulose and organic acid esters of nitro-cellulose or mixtures of the same with organic acid esters of cellulose may be employed, without materially altering the process of manufacture.

Instead of organic acid esters of cellulose, organic acid esters of hydro-cellulose or of oxycellulose, or hydrated cellulose esters may be employed.

Instead of nitro-cellulose and the above mentioned mixtures of the same with organic acid esters of nitro-cellulose and organic acid esters of cellulose I may exclusively employ organic acid esters of cellulose and chloral-alcoholate alone or mixed with chloral-hydrate, with or without the addition of the admixtures usually found in celluloid, in order to obtain a product resembling celluloid and having the properties described above.

Example I: 5 parts by weight of nitro-cellulose and 2 parts of chloral-hydrate are worked up in the known manner with the addition of alcohol or ether.

Example II: 3 parts by weight of cellulose acetate and 2 parts of chloral-alcoholate are intimately mixed together and then com-

pressed, with or without the aid of gentle heating.

I may work also with acetone, acetic ether and other liquid solvents of nitrocellulose. If acetone is used, I may, for instance, mix two parts by weight of nitrocellulose with 1 part by weight of chloralhydrate and then gelatinize the mixture with 3 parts of acetone. The mass thus obtained is then treated further in the known manner.

The same procedure may be adopted, if the nitro-cellulose is partly replaced by acetyl-nitrocellulose, or if instead of nitro-cellulose acetyl-nitrocellulose is exclusively employed.

If instead of chloralhydrate a chloral-alcoholate is employed, either partly or exclusively, no change is necessary in the conditions of working described above.

If it is desired in the above procedure to replace the nitro-cellulose partly by acetyl-cellulose, for instance triacetyl-cellulose, the following process for instance, may be adopted: 3 parts of nitro-cellulose, preferably in the shape of a fine powder, are mixed with 2 parts of chloralhydrate, 6 parts of a 16 per cent. solution of acetyl-cellulose in acetylene-tetrachlorid are added, which correspond to about 1 part of acetyl-cellulose, the mixture is well kneaded and finally gelatinized by means of 3 parts of acetone. The mass thus obtained is then treated further in the known manner. If acetyl-cellulose soluble in acetone be employed, acetone alone may be used as a solvent.

For the manufacture of films and similar products larger quantities of liquefying agents are used and the solution is poured on a suitable base.

I proceed in the same manner, if the solution of the mixture prepared from chloral and cellulose ester is to be used as a lacquer.

Chloral-hydrate may be used in combination with camphor in such proportions, that liquefaction of the two compounds does not take place at ordinary temperature.

Various combinations of camphor or of a camphor-substitute or both with another chloral compound, or with a combination of such compounds, may also be employed.

What I claim is:—

1. The herein described improvement in

the manufacture of products resembling celluloid, which consists in dissolving nitro-cellulose and a chloral-compound without camphor in a suitable solvent and then causing the solvent to evaporate.

2. The herein described improvement in the manufacture of products resembling celluloid, which consists in dissolving nitro-cellulose and chloral-hydrate devoid of cam-

phor in a suitable solvent and then causing the solvent to evaporate.

In witness whereof I have hereunto set my hand in the presence of two witnesses.

DR. LEONHARD LEDERER.

Witnesses:

JULIUS TROGGER,  
PAUL CUBASCH.